# EUROPEAN PATENT SPECIFICATION

(11) **EP 2 629 305 B1**
(45) Date of publication and mention of the grant of the patent: **02.04.2014**
(21) Application number: 12156168.2
(22) Date of filing: 20.02.2012
(51) Int. Cl.: H01B 1/22, H01B 3/47, H01B 3/28

(54) **Composite materials for use in high voltage devices**
Verbundstoffmaterialien zur Verwendung in Hochspannungsvorrichtungen
Matériaux composites pour une utilisation dans des dispositifs haute tension

(43) Date of publication of application: 21.08.2013
(73) Proprietor: ABB Technology AG, 8050 Zürich (CH)
(72) Inventor: Rocks, Jens, CH-8807 Freienbach (CH); Odermatt, Walter, CH-5502 Hunzenschwil (CH)
(74) Representative: ABB Patent Attorneys

(56) References cited:
- EP-A1- 1 775 735
- EP-A1- 1 978 049
- WO-A1-2009/109216
- US-A- 3 573 210

## Description

### Technical Field

The present invention relates generally the field of high-voltage devices and concerns new composite materials and their use in the manufacture of high voltage devices and more particularly of a high voltage device. Such devices are used, e.g., in high-voltage apparatuses like generators or transformers, or in high voltage installations like gas-insulated switchgears.

### Background Art

The main requirements of insulating materials which are used for the manufacture of the above mentioned devices - particularly bushings - are: (i) good electrical insulation (high resistance), (ii) high dielectric strength, (iii) good mechanical properties (i.e., tenacity and elasticity), (iv) they should not be affected by surrounding chemicals. Also, the materials should be non-hygroscopic because the dielectric strength of any material is extremely negatively affected by moisture.

A high-voltage outdoor bushing is a component that is usually used to carry current at high potential from an encapsulated active part of a high-voltage component, like a transformer or a circuit breaker, through a grounded barrier, like a transformer tank or a circuit breaker housing, to a high-voltage outdoor line. Such bushings are typically used in high voltage devices, in particular in switchgear installations or in high-voltage machines, like generators or transformers, for voltages up to several hundred kV.

In order to decrease and control the resulting high electric field, bushings generally comprise a conductor extended along an axis, a condenser core and an electrically insulating polymeric weather protection housing moulded on the condenser core. The condenser core decreases the electric field gradient and distributes the electric field homogeneously along the length of the bushing. Thereby, the condenser core provides a relatively uniform electric field and thus facilitates the electrical stress control.

The condenser core contains an electrically insulating material, and depending on the type of material, there are several kinds of condenser cores. According to the early state of the art, the condenser core of a bushing is typically wound from kraft paper or creped kraft paper as a spacer. According to a more recent alternative, the condenser cores are impregnated either with oil (OIP, oil impregnated paper) or with resin (RIP, resin impregnated paper). RIP bushings showed the advantage that they represent dry (oil free) bushings. The core of an RIP bushing is wound from paper. The resin is then introduced during a heating and vacuum process of the core. However, the disadvantage of impregnated paper bushings is that the process of impregnating the pre-wound stack of paper and metal films with oil or with a resin is a slow process.

The next generation of resin-impregnated cores for bushings is represented by devices in which the bushing has a conductor and a core surrounding the conductor, wherein the core comprises a sheet-like spacer wound in spiral form around the conductor. The spacer is impregnated with an electrically insulating matrix material. By the spiral winding of the spacer, a multitude of neighbouring layers is formed. The core further comprises equalization elements with electrically conductive layers, which are arranged in appropriate radial distances to the axis. The layers have openings, through which openings the matrix material can penetrate. Such a device is disclosed in EP-A-1 798 740.

EP 1 775 735 also discloses electrical insulation systems for high voltage devices.

According to this state of the art, a polyester fabric replaces the paper as a means to give mechanical strength to the condenser core and to support the conducting material which is used for electrical field grading within the condenser core body. Due to the fact that the fabric exhibits an open weave or open knit structure it is possible to achieve an improved impregnation, drying and processing, as compared with paper.

Generally, the fabric should act as a spacer, and therefore fibers of normal thickness or relatively thick fibers have been used, so that the desired volume of the core is obtained without excessive winding and at a reasonable cost.

However, it has been observed that the fibers tend to delaminate from the matrix material in which they are embedded. Accordingly, internal cavities, or free spaces, result between the fibers and the matrix material.

However, the formation of such cavities between the matrix and the fibers may lead to partial discharge and consequently to a potentially fatal failure of the insulation. Even singular flaws in the insulation volume and inhomogeneities at inner material interfaces may compromise the isolation capability. Therefore, there is a desire to reduce the risk of such delaminations reliably.

### Disclosure of the Invention

Accordingly, it is an object to create an insulation material - preferably an insulation material for use in the manufacture of high voltage bushings or other high-voltage devices - that at least reduces the above-mentioned disadvantages, and which particularly shows no - or at least very small - free spaces between the fiber and the cured matrix material. Moreover, it is an object to provide for a method of manufacturing a high-voltage device comprising the above insulation material.

In view of the above, a composite material according to claim 1, its use according to claim 11, a high voltage device according to claim 12, and a method according to claim 14 are provided. Further advantages, features, aspects and details of the invention are evident from the dependent claims, the description and the drawing.

According to one aspect, the above identified problem can be solved at least to some degree by a composite material for use in a high-voltage device having a high-voltage electrical conductor, the composite material being adapted for covering the high-voltage electrical conductor at least partially for grading an electrical field of the high-voltage electrical conductor, the composite material comprising: a polymeric matrix; and at least one fiber embedded in the polymeric matrix, the at least one fiber having an average diameter of less than 500 nm.

According to a further aspect, the composite material is used for the manufacture of a high voltage device.

According to a further aspect, a high voltage device comprises a high-voltage electrical conductor, and the composite material described herein. The composite material covers the conductor at least partially for grading an electrical field of the high-voltage electrical conductor.

According to a further aspect, a method of manufacturing a high-voltage device comprises: providing a high-voltage electrical conductor, winding at least one fiber around the high-voltage electrical conductor, the fibers having an average diameter of less than 500 nm, and embedding the fibers or the fabric in a polymeric matrix. Thereby, a composite material which includes the fibers embedded in the polymeric matrix is obtained.

The diameter of the fibers may be from 20 nm to 500 nm, or even from 50 nm to 500 nm. The lower limit of the average fiber diameter may alternatively even be as high as 80 nm or 100 nm, whereby cost is reduced. With any of the lower limits described herein, the upper limit for the fiber diameter may alternatively be as low as 400 nm or 300 nm, whereby the risk of delamination is further reduced.

As used herein "high voltage device" is defined as a device adapted for carrying a voltage of at least 1 kV AC or 1,5 kV DC through a possibly grounded interface. For example, the voltage rating for a high voltage device may be between about 17.5 kV and about 800 kV. Rated currents may be between 1 kA and 50 kA.

As used herein "fiber" shall mean a single fiber as well as a plurality of fibers. The at least one fiber may form a woven or non-woven fabric. According to one aspect of the invention, the at least one fiber forms at least one sheet-like layer in the polymer matrix.

The fiber used in the manufacture of the composite materials can be made from electrically insulating or electric conductive organic or inorganic materials.

Suitable materials of the fiber comprise organic polymers such as polyolefins - for example polyethylene (PE) or polypropylene -, polyesters, polyamides, aramides, polybenzimidazoles (PBI), polybenzobisoxazoles (PBO), polyphenylene sulphides (PPS), melamine based polymers, polyphenols, polyimides;

Alternatively, the fiber may be from inorganic materials (e.g. alumina or glass), such as S-glass fiber, E-glass fiber, Altex fiber (Al₂O₃ / SiO₂), Nextel fiber (Al₂O₃ / SiO₂ / B₂O₃), quartz, carbon (graphite fibers), basalt fibers (SiO₂ / Al₂O₃ / CaO / MgO), alumina fibers (Almax fiber, Al₂O₃) Boron fibers, Silicon carbide fiber (SiC, SiCN, SiBCN), Beryllium fibers, or fibers from ceramic materials and/or from electrically conductive materials, such as metal or graphite. Also, the fiber(s) may be made from non-conductive materials but coated with at least one electrically conductive or with at least one semi-conductive layer.

Fibers from organic material, in particular from polymers or copolymers, are preferred since the physical properties of organic polymers can be fine tuned so that the polymers - and the fibers which are made from these polymers - can optimally perform for their intended use. Properties that can be fine tuned include, without limitation, particularly Tg (glass transition temperature), molecular weight (both Mₙ and M_{w}), polydispersity index (PDI, the quotient of M_{w}/Mₙ) and degree. For example, the polymers can be designed to show low Tgs are "sticky" and such low-Tg- polymers have beneficial features in that these polymers are more elastic at a given temperature than polymers having higher Tgs.

Also, it is of great advantage to use fibers that have a low or vanishing water uptake, in particular a water uptake that is small compared to the water uptake of cellulose fibers.

As a general aspect, the fibers are provided as single fibers forming a woven layer (fabric) or a non-woven layer. Such single monofilament fibers reduce the risk of delamination more reliably than a bundle of fibers.

The matrix material is a polymer-based material. These polymers can typically be represented by resins on the basis of a silicone, epoxy polymers, hydrophobic epoxy polymers, unsaturated polyesters, in particular poly vinylesters, polyurethanes, poly phenols, polycarbonates, polyether imines (Ultem^{™}), copolymers and/or mixtures thereof. - According to a preferred aspect, the polymers are represented by hydrophobic epoxy polymers.

The at least one fiber may be coated with an adhesion promoting agent which allows the physical or chemical of the at least one fiber attachment to the polymer matrix. Suitable adhesion promoting agents are represented by adhesion promoting organic polymers such as polyvinyl alcohols, polyvinyl acetates (PVA), carboxymethyl cellulose, polyacrylic (PAA) or polymethacrylic acids (PMA), styrene/maleic acid anhydride copolymers poylurethanes, cyanacrylates as well as copolymers and mixtures thereof.

Such polymeric adhesion promoting agents - particularly polyurthanes - provide for the attachment of a great number of fibers which are made from different fiber materials to a variety of polymer matrices. Epoxy polymers form a heat and chemical resistant attachment of the fibers to the matrix; moreover, epoxy polymers form strong bonds and represent good electrical insulators. Polyvinyl acetates (PVA) lead to a connection between the fiber(s) and the matrix having thermoplastic characteristics. Methacrylate polymers adhesion promoting agents form connections between the fiber(s) and the matrix material which exhibit a good impact resistance, flexibility and shear strength. The selection of cyano acrylate polymers result in short cure times, which leads to a short manufacturing time of composite materials or of the high voltage devices.

The fibers may have a mechanically treated surface, in particular a roughened surface, for improved adhesion of the matrix material. The mechanically treated surface may be brushed, etched, coated or otherwise treated. This will further reduce the risk of delamination.

The invention described herein is most advantageously applicable with polymeric fibers, but is also be applicable with other organic or inorganic fiber materials. It is even applicable with fibers which can - due to their chemical characteristics - not form a covalent bond to the matrix material - particularly to the epoxy polymer - or which cannot be impregnated due to their physical structure.

According to another aspect, the matrix material may comprise filler particles. Preferably, the matrix comprises a polymer containing filler particles. The polymer can for example be represented by an epoxy resin, a polyester resin, a polyurethane resin, or another electrically insulating polymer as outlined above. Preferably, the filler particles are electrically insulating or semiconducting. Suitable filler particles can, e.g., be represented by particles selected from inorganic compounds, such as SiO₂, Al₂O₃, BN, AlN, BeO, TiB₂, TiO₂, SiC, Si₃N₄, B₄C or the like, or mixtures thereof. It is also possible to use a mixture of various such particles in the polymer. Preferably, the physical state of the particles is solid.

Compared to a core with un-filled resin as matrix material, there will be less resin in the core, if a matrix material with a filler is used. Accordingly, the time needed to cure a curable monomer or oligomer mixture can be considerably reduced, which reduces the time which is needed to manufacture a high voltage device.

Moreover, it is advantageous if the coefficient of thermal expansion of the filler particles is smaller than the coefficient of thermal expansion of the polymer. If the filler material is chosen accordingly, the thermo-mechanical properties of the high voltage devices are considerably enhanced. A lower coefficient of thermal expansion of the core due to the use of a matrix material together with a filler will lead to a reduced total chemical shrinkage during curing. This enables the production of (near) end-shape devices - or particularly bushings (machining free) - and, therefore, considerably reduces the production time of the high voltage device such as a bushing.

According to a further aspect, the composite material further comprises electrically conductive or semiconductive sheet-like layers dispersed in the matrix as electrical field equialization layers.

According to an aspect alternative to some of the above aspects, the fibers of the composite material described above may be replaced by fibers having a average diameter of more than 500 nm, if the fibers are coated with the above described adhesion promoting agent. Then, the risk of delaminations is reduced solely by the adhesion promoting agent and not by the geometry of the fibers. However, a fiber with less than 500 nm in diameter is preferred. If such a small-radius fiber is combined with the above described adhesion promoting agent, the fiber geometry and the adhesion promoting agent have a synergy effect for reducing the risk of delamination most efficiently.

According to an aspect, the high voltage device described herein is one of the following: a transformer winding of a high-voltage transformer; a current transformer for high voltage application; a high-voltage through-conductor, wherein the composite material is a bushing surrounding the high-voltage through-conductor; a high-voltage cable end termination, wherein the composite material is a cable end insulator surrounding the cable end.

Each of the aspects and embodiment described herein can be combined with other aspects and embodiments, whereby additional aspects and embodiments are obtained. It is intended that all these aspects and embodiments are part of the disclosure herein.

In the following, the exemplary use of the composite materials of the present invention is explained using a bushing as example. However, it will be understood, that the composite materials can be used in a great variety of applications inside as well as outside of the field of high voltage engineering.

### Description of the Drawing

Fig. 1 shows one embodiment of the high-voltage outdoor bushing according to the invention with an axial partial section through the bushing on the right. The described embodiment is meant as example and shall not confine the invention.

The bushing which is shown in Fig. 1 is substantially rotationally symmetric with respect to a symmetry axis 1. In the center of the bushing is arranged a columnar supporting body 2, which is executed as solid metallic rod or a metallic tube. The metallic rod (supporting body 2) is an electric conductor which connects an active part of an encapsulated device, for instance a transformer or a switch, with an outdoor component, for instance a power line.

In an alternative embodiment, the supporting body 2 may be a tube in which the electrical conductor, such as an end of a cable, is received. In this case, the conductor may be guided from below into the supporting body 2 (tube). Generally, the supporting body 2 can be a rod or a tube or a wire. In the following, the supporting body 2 is described as a conductor.

The axis 1 does not need to be a full symmetry axis. The axis 1 is generally defined through the shape of the supporting body 2.

The supporting body 2 is partially surrounded by a core 3, which is substantially rotationally symmetric with respect to the axis 1. The core 3 covers the supporting body 2 between an upper axial end 8 and a lower axial end.

The core 3 is made of the composite material according to an aspect of the present invention. The core 3 comprises an insulating layer 4 of one or more fibers, which is/are wound around the conductor 2. The insulating layer 4 is embedded in and impregnated with a matrix material.

The fiber 4 may be any fiber disclosed herein, having an average diameter of less than 500 nm. For example, a fiber on the basis of polyester may be used. The fiber 4 forms one or more woven or non-woven layers, or sheet-like spacers, which are wound in spiral form around the axis 1. Thus a multitude of neighbouring layers is formed.

The fiber 4 is impregnated with an electrically insulating matrix material. The matrix may be any polymeric matrix disclosed herein. The matrix material may, for example, be a cured polymer-based resin and optionally filled with an inorganic filler powder. For example, the matrix may be an epoxy resin or polyurethane filled with particles of Al₂O₃. Also, in an example, the filler powder comprises approximately 45% by volume of the matrix material before curing. In yet another example, the matrix comprises an epoxy resin which was cured with an anhydride and as filler powder fused silica. The sizes of the fused silica particles can be up to 64 µm and comprise three fractions with different average particle sizes, such as sizes of 2, 12 and 40 µm respectively.

The thermal conductivity of the core in the case of pure (not particle-filled) resin is typically about 0.15 W/mK to 0.25 W/mK. When a particle-filled resin is used, values of at least 0.6 W/mK to 0.9 W/mK or even above 1.2 W/mK or 1.3 W/mK for the thermal conductivity of the bushing core can readily be achieved. The coefficient of thermal expansion can be much smaller when a particle-filled matrix material is used. This results in less thermo-mechanical stress in the bushing core.

Electrically conductive grading insertions, or equalization elements, 5 are arranged between adjacent windings of the tape 4. The grading insertions 5 serve as floating capacitances which homogenize and control the electric field, thereby decreasing the electric field gradient. Generally, the conductive grading insertions 5 are provided as layers which are separate from the fiber layers (the layer defined by the fiber 4). The grading insertions 5 may be formed as respective layers made from fibers coated with an electrically conductive coating. Alternatively or additionally, the grading insertions 5 can be formed as conductive films. The grading insertions 5 (e.g. conductive films) can be continuous or be provided as a plurality of separate parts (e.g. films), which are not connected to each other but which are positioned at a common diameter.

The conductive grading insertions 5 and the fiber 4 may form alternating layers, both being wound spiral-like around the conductor 2. Generally, there can be between two and fifteen fiber layers between neighbouring grading insertion layers. However, it is also possible to have only one, or more than fifteen, fiber layer between neighbouring grading insertion layers.

At a radial end of the bushing, a foot flange 6 is provided, which allows to fix the bushing to a grounded enclosure of the encapsulated device. Under operation conditions the conductor 2 is on high potential, and the condenser core 3 ensures the electrical insulation between the conductor 2 on the one hand and the outside including the flange 6 on the other hand.

Further, an electrically insulating weather protection housing 7 surrounds the core 3 on the outside. The weather protection housing 7 is manufactured from a polymer on the basis of a silicone or a hydrophobic epoxy resin. The housing 7 comprises sheds and is moulded on the condenser core 3 such that it extends from the top of the foot flange 6 along the adjoining outer surface of the condenser core 3 to the upper end 8 of the conductor 2. The housing protects the condenser core 3 from ageing caused by radiation (UV) and by weather and maintains good electrical insulating properties during the entire life of the bushing. The shape of the sheds is designed such, that it has a self-cleaning surface when it is exposed to rain. This avoids dust or pollution accumulation on the surface of the sheds, which could affect the insulating properties and lead to electrical flashover.

An adhesive layer which is deposited on covered surfaces of the parts 2, 3 and 6 improves adhesion of the various components to each other and to the housing 7.

In case that there is an intermediate space between the core 3 and the housing 7, an insulating medium, e.g. an insulating liquid like silicone gel or polyurethane gel, can be provided to fill that intermediate space, or any other space within the bushing.

Next, the manufacturing of the bushing of Fig. 1 is described. First, the supporting body (electrical conductor) 2 is provided and mounted on a winding spool or the like. Then, one or more fibers are wound around the supporting body 2 by rotating the supporting body 2 on the winding spool. The fiber 4 may be any fiber disclosed herein, having an average diameter of less than 500 nm. The fiber 4 may be provided as a woven or non-woven tape-like layer with a width direction extending along the axis 1. The layer may be provided as one or more strips or pieces (axially adjacent to one another and / or on top of one another so that several layers are produced by winding the supporting body 2 about the axis once).

The grading insertions 5 can be wound between two layers of fiber 4. To this purpose, the grading insertions 5 are inserted into the core after certain numbers of windings, so that the grading insertions are arranged in a well-defined, prescribable radial distance to the supporting body 2. Then, the winding process is continued so that the grading insertion 5 in the fabricated bushing lies between two layers of fiber layer 4. Another possibility is to fix the grading insertion 5 to one or more stacked layer(s) of fiber before or during winding.

Instead of winding the fiber 4 on the supporting body 2, it is also possible to wind the fiber 4 on a mandrel, which is removed after finishing the production process. Later the supporting body 2 may be inserted into the hole in the core 3 which is left at the place at which the mandrel was positioned. In that case, the supporting body 2 may be surrounded by some insulating material like an insulating liquid in order to avoid air gaps between the supporting body 2 and the core.

Next, the wound core of the fiber(s) 4 is immersed in the polymeric matrix material. This can be done by applying a vacuum and applying the matrix material to the evacuated fiber (i.e. to the not-yet-finished core) until the fiber is fully impregnated. The impregnation under vacuum takes place at temperatures of typically between 25 °C and 130 °C.

Then, the polymeric matrix material is cured or otherwise hardened, in the case of an epoxy at a temperature of e.g. between 60 °C and 150 °C. Possibly, the matrix material is then also post-cured in order to reach the desired thermo-mechanical properties. Then the core is cooled down, eventually machined, and the flange 6, the insulating envelope 7 and other parts are applied. As a result, a composite material is obtained which includes the fibers embedded in the polymeric matrix material.

The above description mainly relates to a bushing having the composite material according to aspects of the invention. Instead of a bushing, the above description is equally applicable also to other high-voltage devices, some of which have been mentioned herein. These other high-voltage devices can be manufactured in an analogous manner as the bushing described above.

An advantage of the composite material described herein is that the risk of a delamination between the fiber and the matrix material is reduced considerably.

The delamination is believed to be mainly a consequence of the different thermal expansion coefficient of the fibers and polymeric matrix, and of the strong temperature variations during the fabrication of the condenser core, as described above. Namely, the geometry of the enclosed fibers in the matrix material is frozen at a high temperature (e.g. the hotspot temperature in the case of an epoxy resin, or more generally at the reaction temperature of the polymerization process at which the matrix is cured or hardened). Thereafter, the condenser core cools down to room temperature. During this cooling, the fibers and the matrix material undergo a mutually different change in volume and consequently delaminate from each other.

As it turns out, this problem of delamination is significantly reduced when the fibers have a very small diameter of less than 500 nm. This is a unusual diameter for a fiber which should, after all, serve as a spacer. However, this small diameter reduces the length scale on which the different thermal expansion between fiber and matrix material is relevant; and thereby reduces the tensions between fiber and matrix material due to this thermal expansion. As a consequence, even the relatively weak bonding between the fibers and the matrix material is sufficient for avoiding delamination.

In addition, the bonding can be improved by having the fiber coated with an adhesion promoting agent, such as a primer. In particular, the adhesion promoting agent may cause a covalent binding between the fiber and the matrix. In this manner, the adhesion promoting agent further improves the physical or chemical attachment of the fiber to the polymer matrix.

## Claims

1. Composite material for use in a high-voltage device having a high-voltage electrical conductor, the composite material being adapted for covering the high-voltage electrical conductor at least partially for grading an electrical field of the high-voltage electrical conductor, the composite material comprising:
- a polymeric matrix; and
- at least one fiber embedded in the polymeric matrix, the at least one fiber having an average diameter of less than 500 nm.

2. The composite material according to claim 1, wherein the fiber has a diameter from 20 nm to 500 nm, and preferably from 50 to 500 nm.

3. The composite material according to any one of the preceding claims, wherein the at least one fiber is at least one of the following: a plurality of fibers, and a woven or non-woven fabric of the at least one fiber.

4. The composite material according to any one of the preceding claims, wherein the polymeric matrix comprises a resin which comprises an organic or inorganic polymer, such as a silicone, an epoxy polymer, a polyester, a polyurethane, a polyphenole, copolymers thereof; particularly a hydrophobic epoxy polymer, an unsaturated polyester, a polyvinylester, a polyurethane or a polyphenol, polycarbonates, polyether imines (Ultem^{™}), copolymers and/or mixtures thereof and preferably a hydrophobic epoxy polymer.

5. The composite material according to any one of the preceding claims, wherein the fiber is made from an electrically insulating organic or inorganic polymer comprising polyethylene (PE), polyester, polyamide, aramide, polybenzimidazole (PBI), polybenzobisoxazole (PBO),polyphenylene sulphide (PPS), melamine based polymers, polyphenols, polyimides, S-glass fiber, E-glass fiber, Altex fiber (Al₂O₃ / SiO₂), Nextel fiber (Al₂O₃ / SiO₂ / B₂O₃), quartz, carbon (graphite fibers), basalt fiber (SiO₂ / Al₂O₃ / CaO / MgO), alumina (Almax fiber, (Al₂O₃) Boron fiber, Silicon carbide fiber (SiC, SiCN, SiBCN), Beryllium fiber, or ceramic materials and/or from an electrically conductive materials, preferably metal fibers or electrically conductive fibers, preferably (graphite fibers) or fibers which are made from non-conductive materials which are coated with at least one electrically conductive or semi-conductive layers.

6. The composite material according to any one of the preceding claims, wherein the at least one fiber is coated with an adhesion promoting agent which allows the physical or chemical attachment to the polymer matrix.

7. The composite material according to claim 6, wherein the adhesion promoting agent is an organic polymer, preferably selected from the group comprising polyurethanes, epoxyy polymers, polyvinylalcohols, polyvinylacetates, carboxymethyl celluloses, polyacrylic or polymethacrylic acids, styrene/maleic acid anhydride copolymers.

8. The composite material according to any one of the preceding claims, further comprising filler particles dispersed in the polymeric matrix.

9. The composite material according to any one of the preceding claims, the at least one fiber forming at least one sheet-like layer in the polymer matrix.

10. The composite material according to any one of the preceding claims, further comprising electrically conductive or semiconductive sheet-like layers dispersed in the matrix as electrical field equialization layers.

11. Use of the composite material according to any one of the preceding claims for the manufacture of a high voltage device.

12. High voltage device comprising
a high-voltage electrical conductor, and
the composite material according to any one of the preceding claims 1 to 10, wherein
the composite material covers the conductor at least partially for grading an electrical field of the high-voltage electrical conductor.

13. High voltage device according to claim 12, wherein the high-voltage electrical conductor is one of the following:
- a transformer winding of a high-voltage transformer;
- a current transformer for high voltage application;
- a high-voltage through-conductor, wherein the composite material is a bushing surrounding the high-voltage through-conductor;
- a high-voltage cable end termination, wherein the composite material is a cable end insulator surrounding the cable end.

14. Method of manufacturing a high-voltage device, the method comprising:
- providing a high-voltage electrical conductor,
- winding at least one fiber around the high-voltage electrical conductor, the fibers having a naverage diameter of less than 500 nm,
- embedding the fibers or the fabric in a polymeric matrix, thereby obtaining a composite material which includes the fibers embedded in the polymeric matrix.

15. The method according to claim 14, further comprising hardening the polymeric matrix.

## Patentansprüche

1. Verbundmaterial für die Verwendung in einer Hochspannungsvorrichtung mit einem elektrischen Hochspannungsleiter, wobei das Verbundmaterial dafür ausgelegt ist, den elektrischen Hochspannungsleiter wenigstens teilweise zu bedecken, um ein elektrisches Feld des elektrischen Hochspannungsleiters zu glätten, wobei das Verbundmaterial umfasst:
- eine Polymermatrix; und
- wenigstens eine in der Polymermatrix eingebettete Faser, wobei die wenigstens eine Faser einen mittleren Durchmesser von weniger als 500 nm aufweist.

2. Verbundmaterial gemäß Anspruch 1, wobei die Faser einen Durchmesser von 20 nm bis 500 nm aufweist, vorzugsweise von 50 bis 500 nm.

3. Verbundmaterial gemäß einem der vorstehenden Ansprüche, wobei die wenigstens eine Faser wenigstens eines von Folgendem ist: eine Vielzahl von Fasern und ein gewebtes oder nichtgewebtes Gewebe aus der wenigstens einen Faser.

4. Verbundmaterial gemäß einem der vorstehenden Ansprüche, wobei die Polymermatrix ein Harz umfasst, das ein organisches oder anorganisches Polymer, wie z. B. ein Silicon, ein Epoxypolymer, ein Polyester, ein Polyurethan, ein Polyphenol, Copolymere davon, insbesondere ein hydrophobes Epoxypolymer, ein nichtgesättigter Polyester, ein Polyvinylester, ein Polyurethan oder ein Polyphenol, Polycarbonate, Polyetherimine (Ultem^{™}), Copolymere und/oder Gemische davon, vorzugsweise ein hydrophobes Epoxypolymer, umfasst.

5. Verbundmaterial gemäß einem der vorstehenden Ansprüche, wobei die Faser aus einem elektrisch isolierenden organischen oder anorganischen Polymer, umfassend Polyethylen (PE), Polyester, Polyamid, Aramid, Polybenzimidazol (PBI), Polybenzobisoxazol (PBO), Polyphenylensulfid (PPS), melaminbasierte Polymere, Polyphenole, Polyimide, S-Glas-Faser, E-Glas-Faser, Altex-Faser (Al₂O₃/SiO₂), Nextel-Faser (Al₂O₃/SiO₂/B₂O₃), Quarz, Kohlenstoff (Graphitfaser), Basaltfaser (SiO₂/Al₂O₃/CaO/MgO), Aluminiumoxid (Almax-Faser, (Al₂O₃), Borfaser, Siliciumcarbidfaser (SiC, SiCN, SiBCN), Berylliumfaser, oder Keramikmaterialien und/oder aus einem elektrisch leifähigen Material, vorzugsweise Metallfasern oder elektrisch leitfähige Fasern, vorzugsweise (Graphitfasern) oder Fasern aus nichtleitenden Materialien, die mit wenigstens einer elektrisch leitfähigen oder halbleitenden Schicht beschichtet sind, besteht.

6. Verbundmaterial gemäß einem der vorstehenden Ansprüche, wobei die wenigstens eine Faser mit einem haftfördernden Mittel beschichtet ist, das die physikalische oder chemische Befestigung an die Polymermatrix ermöglicht.

7. Verbundmaterial gemäß Anspruch 6, wobei das haftfördernde Mittel ein organisches Polymer ist, vorzugsweise ausgewählt aus der Gruppe umfassend Polyurethane, Epoxypolymere, Polyvinylalkohole, Polyvinylacetate, Carboxymethylcellulosen, Polyacryl- oder Polymethacrylsäuren, Styrol/Maleinsäureanhydrid-Copolymere.

8. Verbundmaterial gemäß einem der vorstehenden Ansprüche, ferner umfassend in der Polymermatrix dispergierte Füllstoffpartikel.

9. Verbundmaterial gemäß einem der vorstehenden Ansprüche, wobei die wenigstens eine Faser wenigstens eine blattartige Schicht in der Polymermatrix bildet.

10. Verbundmaterial gemäß einem der vorstehenden Ansprüche, ferner umfassend elektrisch leitfähige oder halbleitende, blattartige Schichten, die in der Matrix dispergiert sind, als elektrisches-Feld-Ausgleichsschichten.

11. Verwendung des Verbundmaterials gemäß einem der vorstehenden Ansprüche für die Herstellung einer Hochspannungsvorrichtung.

12. Hochspannungsvorrichtung, umfassend
einen elektrischen Hochspannungsleiter und
das Verbundmaterial gemäß einem der vorstehenden Ansprüche 1 bis 10, wobei
das Verbundmaterial den Leiter wenigstens teilweise bedeckt, um ein elektrisches Feld des elektrischen Hochspannungsleiters zu glätten.

13. Hochspannungsvorrichtung gemäß Anspruch 12, wobei der elektrische Hochspannungsleiter eines von Folgendem ist:
- eine Transformatorwicklung eines Hochspannungstransformators;
- ein Stromtransformator für die Hochspannungsanwendung;
- eine Hochspannungs-Durchleitung, wobei das Verbundmaterial eine die Hochspannungs-Durchleitung umgebende Durchführung ist;
- ein Hochspannungskabel-Endabschluss, wobei das Verbundmaterial ein das Kabelende umgebender Kabelendisolator ist.

14. Verfahren zum Herstellen einer Hochspannungsvorrichtung, wobei das Verfahren umfasst:
- Bereitstellen eines elektrischen Hochspannungsleiters,
- Wickeln wenigstens einer Faser um den elektrischen Hochspannungsleiter, wobei die Fasern einen mittleren Durchmesser von weniger als 500 nm aufweisen,
- Einbetten der Fasern oder des Gewebes in eine Polymermatrix, um so ein Verbundmaterial zu erhalten, das die in der Polymermatrix eingebetteten Fasern enthält.

15. Verfahren gemäß Anspruch 14, ferner umfassend Härten der Polymermatrix.

## Revendications

1. Matériau composite pour utilisation dans un dispositif haute tension comportant un conducteur électrique haute tension, le matériau composite étant adapté pour recouvrir au moins partiellement le conducteur électrique haute tension afin de répartir le champ électrique du conducteur électrique haute tension, le matériau composite comprenant :
- une matrice polymère ; et
- au moins une fibre incorporée dans la matrice polymère, l'au moins une fibre ayant un diamètre moyen inférieur à 500 nm.

2. Matériau composite selon la revendication 1, dans lequel la fibre a un diamètre de 20 nm à 500 nm, et de préférence de 50 à 500 nm.

3. Matériau composite selon l'une quelconque des revendications précédentes, dans lequel l'au moins une fibre est l'un au moins des éléments suivants : une pluralité de fibres, et un tissu ou non-tissé de l'au moins une fibre.

4. Matériau composite selon l'une quelconque des revendications précédentes, dans lequel la matrice polymère comprend une résine qui comprend un polymère organique ou inorganique, tel qu'un silicone, un polymère époxyde, un polyester, un polyuréthane, un polyphénol, leurs copolymères ; en particulier un polymère époxyde hydrophobe, un polyester insaturé, un polyester vinylique, un polyuréthane ou un polyphénol, des polycarbonates, des polyétherimines (Ultem^{™}), des copolymères et/ou des mélanges de ceux-ci, et de préférence un polymère époxyde hydrophobe.

5. Matériau composite selon l'une quelconque des revendications précédentes, dans lequel la fibre est constituée d'un polymère organique ou inorganique électriquement isolant comprenant le polyéthylène (PE), le polyester, le polyamide, l'aramide, le polybenzimidazole (PBI), le polybenzobisoxazole (PBO), le polysulfure de phénylène (PPS), les polymères à base de mélamine, les polyphénols, les polyimides, la fibre de verre S, la fibre de verre E, la fibre Altex (Al₂O₃ / SiO₂), la fibre Nextel (Al₂O₃ / SiO₂ / B₂O₃), le quartz, le carbone (fibres de graphite), la fibre de basalte (SiO₂ / Al₂O₃ / CaO / MgO), l'alumine (fibre Almax (Al₂O₃)), la fibre de bore, la fibre de carbure de silicium (SiC, SiCN, SiBCN), la fibre de béryllium, ou de matériaux céramiques et/ou de matériaux électriquement conducteurs, de préférence des fibres métalliques ou des fibres électriquement conductrices, de préférence des fibres de graphite ou des fibres qui sont constituées de matériaux non conducteurs qui sont recouverts d'au moins une couche électriquement conductrice ou semiconductrice.

6. Matériau composite selon l'une quelconque des revendications précédentes, dans lequel l'au moins une fibre est recouverte d'un promoteur d'adhérence qui permet la fixation physique ou chimique à la matrice polymère.

7. Matériau composite selon la revendication 6, dans lequel le promoteur d'adhérence est un polymère organique, de préférence choisi dans le groupe comprenant les polyuréthanes, les polymères époxydes, les alcools polyvinyliques, les polyacétates de vinyle, les carboxy-méthylcelluloses, les acides polyacryliques ou poly-méthacryliques, et les copolymères styrène/anhydride d'acide maléique.

8. Matériau composite selon l'une quelconque des revendications précédentes, comprenant en outre des particules de charge dispersées dans la matrice polymère.

9. Matériau composite selon l'une quelconque des revendications précédentes, l'au moins une fibre formant au moins une couche en forme de feuille dans la matrice polymère.

10. Matériau composite selon l'une quelconque des revendications précédentes, comprenant en outre des couches en forme de feuille électriquement conductrices ou semi-conductrices dispersées dans la matrice en tant que couches d'égalisation du champ électrique.

11. Utilisation du matériau composite selon l'une quelconque des revendications précédentes pour la fabrication d'un dispositif haute tension.

12. Dispositif haute tension comprenant
un conducteur électrique haute tension, et
le matériau composite selon l'une quelconque des revendications 1 à 10 précédentes, dans lequel
le matériau composite recouvre au moins partiellement le conducteur pour répartir le champ électrique du conducteur électrique haute tension.

13. Dispositif haute tension selon la revendication 12, dans lequel le conducteur électrique haute tension est l'un des éléments suivants :
- un enroulement de transformateur d'un transformateur haute tension ;
- un transformateur de courant pour une application haute tension ;
- un conducteur traversant haute tension dans lequel le matériau composite est une traversée entourant le conducteur traversant haute tension ;
- une terminaison d'extrémité de câble haute tension dans laquelle le matériau composite est un isolant d'extrémité de câble entourant l'extrémité de câble.

14. Procédé de fabrication d'un dispositif haute tension, le procédé comprenant :
- l'obtention d'un conducteur électrique haute tension,
- l'enroulement d'au moins une fibre autour du conducteur électrique haute tension, les fibres ayant un diamètre moyen inférieur à 500 nm,
- l'incorporation des fibres ou du tissu dans une matrice polymère pour obtenir ainsi un matériau composite qui comprend les fibres incorporées dans la matrice polymère.

15. Procédé selon la revendication 14, comprenant en outre le durcissement de la matrice polymère.
